

Sept. 10, 1968

E. J. DULIS ET AL

3,401,036

VALVE STEEL

Filed Aug. 31, 1967

2 Sheets-Sheet 1

FIG. 1.



INVENTORS.  
EDWARD J. DULIS and  
AUGUST KASAK

By *Clair L. Mullens*  
Attorney

Sept. 10, 1968

E. J. DULIS ET AL

3,401,036

VALVE STEEL

Filed Aug. 11, 1967

2 Sheets-Sheet 2



FIG. 2.



FIG. 3.



INVENTORS.  
EDWARD J. DULIS &  
AUGUST KASAK  
By *Clarendon, Muller, Jr.*  
Attorney

1

3,401,036  
VALVE STEEL

Edward John Dulis, Pittsburgh, and August Kasak, Bridgeville, Pa., assignors to Crucible Steel Company of America, Pittsburgh, Pa., a corporation of New Jersey

Continuation-in-part of application Ser. No. 616,793, Feb. 17, 1967. This application Aug. 11, 1967, Ser. No. 660,007

4 Claims. (Cl. 75—128)

## ABSTRACT OF THE DISCLOSURE

This patent relates to valve steels having an excellent combination of properties with respect to (1) lead oxide corrosion resistance, (2) high-temperature creep strength, (3) machinability, (4) ingot soundness and (5) hot-workability. More specifically, this patent discloses that the above-mentioned desirable results are obtained in certain chromium-containing austenitic stainless steels by using compositions that exhibit the following features: (1) the use of a carbon content within a restricted range of about 0.22% to 0.5%, (2) the use of silicon contents of 0.05 to 0.25%, (3) the use of a strong-carbide-forming strengthening element such as columbium, titanium, tantalum, molybdenum, or tungsten, singularly or in combination, columbium being preferred, within the range of 0.02 to 0.75%, (4) the optional use of boron up to 0.025% and preferably 0.00005 to 0.025%, (5) the use of nitrogen in amounts up to 0.25%, (6) the use of sulfur in substantial amounts up to 0.25%, (7) the use of copper in amounts up to about 3%, (8) chromium of 16 to 22%, (9) nickel 4 to 15%, (10) manganese of 2 to 8%, (11) with the sum of manganese plus nickel within the range of 8 to 20% and the sum of carbon plus nitrogen within the range of .025 to 0.6%.

This application is a continuation-in-part of our earlier filed copending application Ser. No. 616,793 filed Feb. 17, 1967, now abandoned, which is in turn a continuation-in-part of our application Ser. No. 417,240, filed Dec. 9, 1964, which is now abandoned.

This invention relates to high-temperature stainless steel especially suitable for the manufacture of valves, valve parts, and other internal-combustion-engine components intended for use in hot, corrosive atmospheres.

Among the objects of our invention is the provision of strong, tough, and durable stainless steel, and various internal-combustion-engine valves and engine components fashioned of the same for elevated-temperature use, which steel products function in a highly satisfactory manner in such fields as passenger-car, truck, aircraft, diesel and marine-vessel engine use, and which offer both great hardness at the high temperatures encountered in such use and substantial resistance, in the heated condition, to hot corrosive atmospheres such as those containing the combustion products of anti-knock gasolines, e.g., of the tetraethyl lead variety. In addition, the steel is characterized by good workability at the prevailing hardness levels.

Numerous metallurgical compositions have hitherto been used, or proposed for use, in making valves for internal-combustion engines, and especially for internal-combustion-engine exhaust valves, but the steels of our invention possess a combination of properties that, for certain purposes, makes them more suitable than any prior-art steel. Two important properties sought in a stainless steel for internal-combustion-engine exhaust valves are (1) resistance to corrosion by lead-containing fuel-combustion products, and (2) high-temperature stretch resistance (creep strength). Perhaps the foremost of the steels presently used for such purposes is a steel contain-

2

ing about 21% chromium, 4% nickel, 9% manganese, 0.50% carbon, 0.40% nitrogen, 0.25% maximum silicon, and the balance substantially iron. Of the iron-base materials hitherto known which exhibit sufficient creep strength to suit them for use in exhaust valves, this steel, called "21-4N," exhibits the greatest resistance to corrosion by lead-containing fuel-combustion products. The lead oxide crucible test is presently the best laboratory method for preliminary evaluation of the corrosion resistance of exhaust-valve alloys. In the performance of this test, specimens of 0.444 inch in diameter by 0.444 inch long are weighed, placed in a magnesia crucible with 40 grams of lead oxide, and heated to 1675° F. for one hour. Specimens are then cooled to room temperature, cleaned, and weighed again. The loss in weight per unit surface area expresses the relative corrosion resistance of the alloy. In such a test, the above-mentioned "21-4N" alloy exhibits a weight loss of 15 to 19 grams per square decimeter per hour. The preferred steels according to our invention exhibit weight-loss values considerably lower, on the order of 8 to 10 grams per square decimeter per hour, yet our steels are not only less expensive to produce than the "21-4N" alloy but also exhibit a stretch resistance (creep strength) better than that of many other known alloys for use in exhaust valves and better than or not substantially inferior to the values for the "21-4N" alloy.

A further disadvantage of the "21-4N" alloy now in common use is that it is quite difficult to machine. It is known that sulfur improves machinability of austenitic stainless steel and other steels, and that at the same time, it tends to make the steel difficult to hot work; with the known "21-4N" steel, only relatively small amounts, such as about 0.07%, of sulfur can be added to improve the machinability of the steel while still avoiding undue hot working difficulties. Machinability is an important property in a valve steel; the usual practice in the making of exhaust valves for automotive engines involves a two-step hot forming of a cylindrical slug of steel to give it the usual stem and poppet valve head, permitting the hot-formed piece to cool, and then finish machining the valve stem and face to a desired size. A final machining operation is important in order to obtain valves of uniform dimensions. The temperature to which the cylindrical slugs are heated necessarily varies somewhat, so that the amount of contraction obtained upon cooling differs from one valve to the next; moreover, scale forms on the valves as they are cooling and must be removed. The prior art has not furnished a valve steel with good creep strength and good lead oxide corrosion resistance and, at the same time, anything more than marginal machinability.

Yet another advantage of the steel of our invention over conventional valve steels, and particularly "21-4N," is that our steel exhibits good hot-hardness in combination with good hot-workability. In the manufacture of valves for this purpose, it is customary to form the same by a hot-forging operation, typically at a temperature of, for example, 2100° F. Hence, it is desirable that the steel have good hardness at these high temperatures for good performance during service and yet permit forging to the required valve shape without undue resistance to material flow.

The steel of our invention overcomes the above-discussed disadvantages with respect to conventional valve steels and provides other advantages, which will be apparent from the following description and drawings, in which:

FIGURE 1 is a bar graph showing the desirable combination of hardness and hot-workability achieved with our steel by observing our limitations with respect to nitrogen content as compared with conventional stainless steels, particularly "21-4N";

FIGURE 2 is a graph showing the effects of manganese and nickel with respect to providing the steel of our invention with a fully austenitic structure;

FIGURE 3 is a graph showing the relative austenite and martensite percentages at varying levels of manganese and nickel; and

FIGURE 4 is a bar graph showing the effects of various strengthening elements on the creep strength (stretch resistance) of steels of our invention that were austenitized at 2150° F. for one hour, water quenched and tempered at 1400° F. for eight hours.

New austenitic stainless valve steels having improved hot-hardness, hot-workability and machinability as compared with the "21-4N" steel and other conventional stainless steels, together with lead oxide corrosion resistance and creep strength at least about as good as "21-4N" steel, and in some instances, substantially better results as respects those properties, are obtained by making a steel with about 16% to 22% chromium, sufficient nickel and manganese to make the steel completely austenitic, 0.05 to 0.25% silicon, about 0.22% to 0.5% carbon, and a strengthening addition of a carbide-forming element selected from the group consisting of columbium, tantalum, molybdenum, tungsten, and titanium, with columbium being preferred, and balance of the steel being iron, impurities in small amounts not substantially detrimentally affecting the properties, and in some instances, small amounts of other elements such as boron, copper, and sulfur, which may be added in particular cases to improve the properties of the steel further in certain respects. Use of the carbon-content range indicated above is important for obtaining lead oxide corrosion resistance and strength.

The optional addition of boron to the steel of the invention serves to improve the creep strength. The addition of nitrogen in combination with a controlled carbon content provides an optimum combination of hot-workability and hardness. Sulfur may be added to improve machinability. Also, if desired, copper may be added to further improve the creep strength.

The following Table I presents the composition limits, in percent, of steels according to our invention:

TABLE I

|                                                                                                                                         |             |
|-----------------------------------------------------------------------------------------------------------------------------------------|-------------|
| Carbon -----                                                                                                                            | 0.22-0.5    |
| Chromium -----                                                                                                                          | 16-22       |
| Silicon -----                                                                                                                           | 0.05-0.25   |
| Nickel -----                                                                                                                            | 4-15        |
| Manganese -----                                                                                                                         | 2-8         |
| Manganese+nickel -----                                                                                                                  | 8-20        |
| Boron -----                                                                                                                             | Up to 0.025 |
| Sulfur -----                                                                                                                            | Up to 0.25  |
| Nitrogen -----                                                                                                                          | Up to 0.25  |
| Carbon+nitrogen -----                                                                                                                   | 0.25 to 0.6 |
| Copper -----                                                                                                                            | Up to 3     |
| At least one carbide-forming element selected from the group consisting of columbium, molybdenum, tungsten, titanium and tantalum ----- | 0.02-0.75   |
| Iron -----                                                                                                                              | Balance     |

In addition, boron may be present in an amount within the range of 0.00005 to 0.025%. Also, the preferred carbide-forming element is columbium, and such may preferably be present in an amount within the range of 0.05 to 0.25%. Columbium may be present within this range with tantalum within the range of 0.005 to 0.25%. To insure good hot-workability, it is preferred that the nitrogen limit be 0.2%. The steel in accordance with the invention is fully austenitic and substantially free of ferrite.

With carbon contents too low, the strength of the steel is inadequate, and with carbon contents too high no benefit is observed and the steel tends to become difficult to hot-work. The optimum carbon content for this purpose is about 0.357. The carbon content also influences the lead oxide corrosion resistance, optimal values being observed at a carbon content of about 0.36%. It must also be borne in mind that carbon is an austenite-promoting

element. With carbon contents too low, the steel will become partially ferritic unless compensating increases are made in the contents of other austenite-promoting elements.

As respects silicon, the resistance of the steel to corrosion in the presence of the products of combustion of lead-containing fuels is substantially lowered if too much silicon is used. Hence, for use in valves of engines burning leaded fuels, steels containing not over 0.25% silicon, and still more desirably not more than 0.12%, are preferred.

As respects chromium, the steel must contain sufficient of this element to insure the stainless character of the steel, but the use of an amount too great must be avoided in order to prevent the formation of substantial amounts of ferrite and/or sigma phase, which would detrimentally affect the creep resistance of the steel.

As respects nickel, the steel must contain an amount sufficient to insure that the steel will possess an essentially austenitic microstructure, which is required for good creep-strength properties. The use of amounts of nickel greater than those indicated above is without substantial benefit justifying the addition and is contraindicated on account of cost.

As respects columbium, a small addition of this element, or of another appropriate carbide-forming element is required in order to achieve adequate creep strength. The use of amounts of columbium greater than that indicated above is considered undesirable because there is no observed improvement in properties that would justify the cost of using more columbium.

When they are used in place of, or in addition to, columbium, the elements titanium, tantalum, molybdenum, and tungsten are generally to be employed in substantially equivalent amounts on the basis of their atomic weights. That is, 0.1% columbium is equivalent to 0.05% of titanium, or 0.2% of tantalum, or 0.1% of molybdenum, or 0.2% of tungsten. As will be explained below, however, our data with respect to titanium show an anomaly; when titanium is used, it is preferred to use a relatively large amount, such as about 0.36%.

As respects boron, the use of this element is optional, but to provide better creep strength, it is desirable to include an effective addition of boron. The use of quantities greater than those indicated above may cause incipient grain-boundary melting at temperatures of use. Amounts of boron up to 0.1% have a favorable effect upon creep strength, but boron additions of more than about 0.04% tend to worsen resistance of the steel to corrosion by lead oxide, so that it is preferable that the boron not exceed 0.025%.

The primary role of manganese in the steel, and particularly the combination of manganese and nickel, is to control the phase relationships so that an essentially fully austenitic structure is maintained during heat treatment and service. The presence of delta ferrite and/or martensite in the structure has an adverse effect on the stretch resistance of the steel. For this purpose, at least 4% nickel is necessary to prevent the formation of delta ferrite at solution annealing temperatures, e.g., 2150° F., (FIGURE 2). Manganese alone is not effective for this purpose; however, manganese is effective for the purpose of stabilizing the austenitic structure against transformation to martensite when used in combination with nickel (FIGURE 3). Without manganese, at least about 8.5% nickel is necessary for a stable structure. With 4% nickel, at least 5% manganese is needed for a stable structure.

The nitrogen content, in combination with the carbon content, must be controlled to achieve the desired combination of hardness and hot-workability (FIGURE 1). Although the hardness of the steel increases with increasing nitrogen at a given carbon level, e.g., about 0.30%, when the nitrogen content is increased substantially above 0.25 percent the hot-workability of the steel is substantially decreased. As may be seen from FIGURE 1, at

about 0.21% nitrogen, in combination with a carbon content of about 0.31%, the hot-workability of the steel is far superior to that of the conventional "21-4N." When nitrogen is increased to 0.31%, with carbon remaining substantially the same, the hardness is only slightly improved, e.g., increased from 28 R<sub>c</sub> to 30 R<sub>c</sub>; however, the hot-workability is decreased to that typically exhibited by "21-4N." At even higher nitrogen levels, e.g., 0.53 and 0.63%, the hot-workability is substantially decreased over that of "21-4N."

These data presented in FIGURE 1 were obtained by investigating the following steels:

10

The effect of using various strengthening elements (columbium, vanadium, titanium, zirconium, tantalum, molybdenum, tungsten, and aluminum) upon the lead oxide corrosion resistance of steels of this kind was studied, comparison being made with the known "21-4N" steel and with a steel consisting of 21% chromium, 6% manganese, 6% nickel, 0.35% carbon, balance iron, i.e., a steel that would be in accordance with the instant invention, save for the fact that it contains no strengthening-element addition. This steel, designated 1733, is not suitable as a valve steel, exhibiting a plastic strain of 1.62% after 100 hours at 1350° F. under a stress of 16,000 p.s.i. as com-

| Steel  | Heat  | C    | Mn   | S     | Si   | Cr    | Ni    | Cb    | B     | N     | Other   | C+N   |
|--------|-------|------|------|-------|------|-------|-------|-------|-------|-------|---------|-------|
| 65-175 | 1716  | 0.34 | 5.95 | 0.061 | 0.07 | 20.00 | 5.87  | 0.11  | 0.001 | 0.03  | -----   | 0.37  |
| 66-257 | 1x32  | 0.31 | 5.97 | 0.055 | 0.15 | 20.24 | 5.89  | 0.08  | 0.001 | 0.14  | -----   | 0.45  |
| 66-258 | 1x33  | 0.28 | 5.85 | 0.059 | 0.17 | 20.19 | 5.87  | 0.10  | 0.001 | 0.21  | -----   | 0.49  |
| 66-259 | 1x34  | 0.31 | 5.88 | 0.058 | 0.14 | 20.34 | 5.89  | 0.11  | 0.001 | 0.31  | -----   | 0.62  |
| 66-260 | 1x35  | 0.31 | 6.04 | 0.057 | 0.14 | 20.14 | 5.93  | 0.11  | 0.001 | 0.37  | -----   | 0.68  |
| 66-261 | 1x36  | 0.37 | 5.74 | 0.056 | 0.14 | 20.29 | 5.95  | 0.11  | 0.001 | 0.53  | -----   | 0.90  |
| 66-262 | 1x37  | 0.30 | 6.08 | 0.055 | 0.16 | 20.29 | 5.87  | 0.09  | 0.001 | 0.63  | -----   | 0.93  |
| T304   | 39273 | 0.04 | 1.32 | 0.020 | 0.51 | 18.53 | 8.87  | ----- | ----- | ----- | 2.40 Mo | ----- |
| T316   | 10242 | 0.05 | 1.67 | 0.020 | 0.28 | 16.44 | 13.24 | ----- | ----- | ----- | -----   | ----- |
| 21-4N  | 49271 | 0.57 | 9.25 | 0.046 | 0.16 | 20.87 | 4.23  | ----- | ----- | 0.40  | -----   | 0.97  |

For the purposes of this evaluation, 0.65 in. square by 6 in. long specimens of the above steels were hot-rolled in six passes to nominally 0.11 in. long by 1 in. wide flats by a reduction about 25% per rolling pass by the use of 13.5 in. diameter work-rolls. The roll-separating force, entry thickness and exit width of the specimens were measured. These data were used to obtain the flow-stress values presented in FIGURE 1 of the drawings by means of a standard computer technique utilizing the well-known Hill-Longman roll-separating force equation, which is a measure of hot-workability.

As respects sulfur, a noticeable improvement in machinability is obtained with amounts of sulfur as small as 0.05%. Although amounts as large as 0.25% can be used, the improvement in machinability obtained by adding sulfur levels off at slightly above this amount. Hence, amounts in substantial excess of said amount should not be used.

Copper improves the creep strength of the steels.

It has been discovered, moreover, that additions of vanadium, aluminum and zirconium worsen the creep strength of the steel, in comparison to the same steel without any addition of a strengthening element as may be seen from the data presented in FIGURE 4. These steels, varying in composition only with respect to the strengthening element, were creep tested for relative stretch resistance at a temperature of 1350° F. under 16,000 p.s.i. for 100 hours. In these tests the resulting plastic strain (permanent set) is the evaluating criterion. Low plastic-strain values (in percent) are indicative of good creep strength (stretch resistance).

25 paired with a plastic strain of 0.56% in the "21-4N" steel under the same conditions; but its performance in lead oxide corrosion resistance tests gives a valuable indication of the effect of the addition of the various strengthening elements mentioned above upon the property of lead oxide corrosion resistance. Our tests show that all the above-mentioned strengthening elements were detrimental, more or less, to the lead oxide corrosion resistance. Titanium and zirconium impaired the lead oxide corrosion resistance of the 1733 steel to the point where there was no improvement in comparison with the "21-4N" steel. The result with an addition of aluminum in the amount of about 0.23% was nearly as unfavorable. Tantalum additions of 0.12% and 1.57% gave the same result, as did the additions of vanadium. Additions of molybdenum, tungsten and columbium were less detrimental and left the steel with lead oxide corrosion resistance substantially superior to that of the "21-4N" steel.

40 As explained above, only with small additions of columbium was there a substantial improvement over "21-4N" steel in creep strength, and the same small addition of columbium at the same time, yielded a substantial improvement in lead oxide corrosion resistance, for which reason columbium is a preferred strengthening element. It is important, however, not to lose sight of the fact that the improved lead oxide corrosion resistance of 1733 and the same steel with an addition of 0.11% columbium is also in part dependent upon the low nitrogen content of those steels.

55 Data tending to substantiate the statements made above are presented in the following tables, from which the value of the invention will be further apparent.

TABLE II.—COMPOSITIONS AND RESULTS OF LEAD-OXIDE CORROSION TEST

| Heat No. | C    | Mn    | S     | Si   | Cr    | Ni    | Cb   | B     | N     |
|----------|------|-------|-------|------|-------|-------|------|-------|-------|
| 3230     | 0.20 | 1.33  | 1 NA  | 0.08 | 20.15 | 15.85 | 0.13 | 0.001 | 0.004 |
| 3229     | 0.29 | 1.41  | 1 NA  | 0.10 | 20.15 | 15.95 | 0.12 | 0.001 | 0.007 |
| 3103     | 0.36 | 1.35  | 1 NA  | 0.10 | 20.32 | 15.80 | 0.09 | 0.001 | 0.005 |
| 3168     | 0.45 | 1.29  | 1 NA  | 0.07 | 19.92 | 15.58 | 0.10 | 0.002 | 0.005 |
| 3169     | 0.71 | 0.86  | 1 NA  | 0.06 | 19.97 | 15.52 | 0.11 | 0.001 | 0.003 |
| 3170A    | 1.00 | 1.33  | 1 NA  | 0.05 | 20.02 | 15.94 | 0.12 | 0.001 | 0.005 |
| 3260     | 0.36 | 1.27  | 1 NA  | 0.10 | 20.28 | 15.95 | 0.13 | 1 NA  | 0.005 |
| 3261     | 0.36 | 1.30  | 1 NA  | 0.08 | 20.10 | 16.10 | 1 NA | 1 NA  | 0.004 |
| 1569     | 0.35 | 1.42  | 0.013 | 0.09 | 20.52 | 3.08  | 0.12 | 0.003 | 0.01  |
| 1570     | 0.34 | 1.38  | 0.011 | 0.10 | 20.46 | 5.06  | 0.15 | 0.003 | 0.01  |
| 1571     | 0.33 | 1.40  | 0.014 | 0.09 | 20.38 | 6.98  | 0.07 | 0.002 | 0.01  |
| 1572     | 0.32 | 1.34  | 0.011 | 0.10 | 20.40 | 8.92  | 0.08 | 0.003 | 0.01  |
| 1573     | 0.33 | 1.37  | 0.011 | 0.07 | 20.34 | 11.10 | 0.10 | 0.002 | 0.02  |
| 1574     | 0.33 | 1.40  | 0.012 | 0.08 | 20.52 | 12.94 | 0.10 | 0.002 | 0.02  |
| 1575     | 0.33 | 1.30  | 0.012 | 0.08 | 20.32 | 15.75 | 0.11 | 0.005 | 0.02  |
| 1577     | 0.34 | 14.13 | 0.008 | 0.08 | 20.12 | 3.03  | 0.06 | 0.001 | 0.01  |
| 1578     | 0.34 | 10.00 | 0.014 | 0.10 | 19.96 | 6.88  | 0.08 | 0.001 | 0.02  |
| 1604     | 0.33 | 6.20  | 0.016 | 0.08 | 20.06 | 6.30  | 0.08 | 0.002 | 0.02  |
| 1715     | 0.33 | 6.11  | 0.055 | 0.09 | 19.98 | 5.71  | 0.02 | 0.001 | 0.03  |
| 1716     | 0.34 | 5.95  | 0.061 | 0.07 | 20.00 | 5.87  | 0.11 | 0.001 | 0.03  |
| 1717     | 0.35 | 6.03  | 0.052 | 0.12 | 19.80 | 5.85  | 0.62 | 0.001 | 0.04  |
| 1733     | 0.35 | 6.16  | 0.049 | 0.08 | 19.80 | 5.83  | 1.01 | 0.001 | 0.02  |

TABLE II—Continued

| Heat No.          | C     | Mn   | S     | Si   | Cr    | Ni   | Cb                | B                  | N     |
|-------------------|-------|------|-------|------|-------|------|-------------------|--------------------|-------|
| 1714A             | 0.30  | 5.83 | 0.052 | 0.08 | 20.25 | 5.90 | <sup>1</sup> 0.01 | 0.0005             | 0.04  |
| 1716A             | 0.38  | 5.83 | 0.051 | 0.08 | 20.25 | 5.90 | 0.32              | 0.001              | 0.05  |
| 1718A             | 0.36  | 5.83 | 0.046 | 0.09 | 20.20 | 5.90 | 0.11              | <sup>1</sup> 0.005 | 0.05  |
| 1719A             | 0.36  | 5.83 | 0.056 | 0.10 | 20.25 | 5.93 | 0.12              | 0.003              | 0.05  |
| 1720A             | 0.36  | 5.73 | 0.048 | 0.10 | 20.25 | 5.90 | 0.11              | 0.029              | 0.05  |
| 1647              | 0.192 | 5.98 | 0.058 | 0.09 | 19.90 | 5.86 | 0.12              | 0.002              | 0.02  |
| 1643              | 0.27  | 5.98 | 0.052 | 0.09 | 20.24 | 5.84 | 0.08              | 0.001              | 0.02  |
| 1648              | 0.56  | 5.80 | 0.056 | 0.08 | 20.34 | 5.80 | 0.11              | 0.001              | 0.03  |
| 1649              | 0.96  | 5.96 | 0.057 | 0.07 | 20.32 | 5.76 | 0.11              | 0.001              | 0.03  |
| 21-4N             | 0.55  | 9.0  | 0.07  | 0.15 | 21.00 | 4.0  | <sup>1</sup> NA   | <sup>1</sup> NA    | 0.40  |
|                   |       |      |       |      |       |      |                   | V                  |       |
| 1721A             | 0.34  | 6.05 | 0.054 | 0.09 | 20.46 | 5.92 | 0.23              | 0.002              | 0.014 |
| 1722A             | 0.35  | 5.75 | 0.057 | 0.10 | 20.25 | 5.82 | 0.63              | 0.002              | 0.017 |
|                   |       |      |       |      |       |      |                   | Zr                 |       |
| 1723A             | 0.35  | 5.87 | 0.057 | 0.09 | 20.22 | 5.87 | 0.20              | 0.002              | 0.024 |
| 1724A             | 0.35  | 5.84 | 0.056 | 0.09 | 20.27 | 5.93 | 1.19              | 0.003              | 0.015 |
|                   |       |      |       |      |       |      |                   | Ti                 |       |
| 1725A             | 0.35  | 5.64 | 0.058 | 0.12 | 20.46 | 5.89 | 0.06              | 0.002              | 0.025 |
| 1726A             | 0.35  | 5.80 | 0.056 | 0.11 | 20.13 | 5.96 | 0.36              | 0.002              | 0.014 |
|                   |       |      |       |      |       |      |                   | Ta                 |       |
| 1727A             | 0.35  | 5.74 | 0.055 | 0.09 | 20.35 | 5.92 | 0.12              | 0.002              | 0.024 |
| 1728A             | 0.34  | 5.59 | 0.052 | 0.11 | 19.76 | 5.91 | 1.57              | 0.002              | 0.019 |
|                   |       |      |       |      |       |      |                   | Mo                 |       |
| 1729              | 0.36  | 5.92 | 0.051 | 0.08 | 20.12 | 5.87 | 0.10              | 0.001              | 0.03  |
| 1730              | 0.37  | 5.68 | 0.050 | 0.08 | 19.70 | 5.85 | 0.93              | 0.001              | 0.02  |
|                   |       |      |       |      |       |      |                   | W                  |       |
| 1731              | 0.33  | 5.96 | 0.054 | 0.08 | 19.96 | 5.77 | 0.19              | 0.001              | 0.02  |
| 1732              | 0.33  | 5.66 | 0.054 | 0.09 | 19.10 | 5.79 | 1.90              | 0.001              | 0.02  |
|                   |       |      |       |      |       |      |                   | Al                 |       |
| 1734              | 0.34  | 6.01 | 0.060 | 0.10 | 20.24 | 5.93 | 0.23              | 0.001              | 0.03  |
|                   |       |      |       |      |       |      |                   | Cb                 |       |
| 1812              | 0.33  | 5.76 | 0.17  | 0.12 | 19.72 | 5.87 | 0.11              | 0.001              | 0.03  |
| 1813              | 0.34  | 5.60 | 0.22  | 0.09 | 19.67 | 5.89 | 0.11              | 0.001              | 0.02  |
| 1857              | 0.35  | 5.67 | 0.29  | 0.07 | 20.06 | 5.88 | 0.10              | 0.001              | 0.02  |
| 1858              | 0.36  | 5.74 | 0.35  | 0.07 | 20.31 | 5.94 | 0.10              | 0.001              | 0.01  |
| 1814 <sup>2</sup> | 0.33  | 5.94 | 0.086 | 0.11 | 20.18 | 5.91 | 0.12              | 0.001              | 0.03  |
| 1x35              | 0.31  | 6.04 | 0.06  | 0.14 | 20.34 | 5.89 | 0.11              | 0.001              | 0.37  |

<sup>1</sup> None added.<sup>2</sup> Contained also 1.92% copper.

TABLE II—Continued

TABLE III—RESULTS OF CREEP AND CREEP-RUPTURE TESTS AT 1,350° F. UNDER A STRESS OF 16,000 P.S.I.<sup>1</sup>

| Heat No. | Weight loss after immersion in molten PbO for 1 hr. at 1675° F. (g./in. <sup>2</sup> ) | Heat No. | Weight loss after immersion in molten PbO for 1 hr. at 1675° F. (g./in. <sup>2</sup> ) | 50 |       | Heat No. | Plastic strain after 100-hr. exposure, percent | Rupture life, hours | Heat No. | Plastic strain after 100-hr. exposure, percent | Rupture life, hours |
|----------|----------------------------------------------------------------------------------------|----------|----------------------------------------------------------------------------------------|----|-------|----------|------------------------------------------------|---------------------|----------|------------------------------------------------|---------------------|
|          |                                                                                        |          |                                                                                        | 55 | 50    |          |                                                |                     |          |                                                |                     |
| 3230     | 0.83                                                                                   | 1720A    | 1.02                                                                                   | 55 | 3230  | 2.45     | 200                                            | 1719A               | 0.34     | N.D.                                           |                     |
| 3229     | 0.85                                                                                   | 1647     | 0.68                                                                                   |    | 3229  | 1.85     | N.D.                                           | 1720A               | 0.31     | N.D.                                           |                     |
| 3103     | 0.64                                                                                   | 1743     | 0.59                                                                                   |    | 3103  | 0.66     | 402                                            | 1647                | 1.33     | N.D.                                           |                     |
| 3168     | 0.73                                                                                   | 1648     | 1.14                                                                                   |    | 3168  | 1.34     | 234                                            | 1648                | 3.54     | N.D.                                           |                     |
| 3169     | 0.88                                                                                   | 1649     | 0.95                                                                                   |    | 3169  | 1.39     | 204                                            | 1649                | 17.4     | N.D.                                           |                     |
| 3170A    | 0.96                                                                                   | 21-4N    | 1.00                                                                                   |    | 3170A | 2.03     | N.D.                                           | 21-4N               | 0.56     | N.D.                                           |                     |
| 3260     | 0.72                                                                                   | 1721A    | 0.76                                                                                   |    | 3260  | 1.96     | 184                                            | 1721A               | 3.62     | N.D.                                           |                     |
| 3261     | 0.82                                                                                   | 1722A    | 0.86                                                                                   |    | 3261  | 8.80     | 124                                            | 1722A               | 2.39     | N.D.                                           |                     |
| 1569     | 0.88                                                                                   | 1723A    | 0.94                                                                                   |    | 1569  | 1.22     | N.D.                                           | 1723A               | 1.55     | N.D.                                           |                     |
| 1570     | 0.85                                                                                   | 1724A    | 1.06                                                                                   |    | 1570  | 1.19     | N.D.                                           | 1724A               | 2.30     | N.D.                                           |                     |
| 1571     | 1.03                                                                                   | 1725A    | 0.87                                                                                   |    | 1571  | 0.67     | N.D.                                           | 1725A               | 3.08     | N.D.                                           |                     |
| 1572     | 1.01                                                                                   | 1726A    | 1.02                                                                                   |    | 1572  | 0.66     | N.D.                                           | 1726A               | 0.66     | N.D.                                           |                     |
| 1573     | 0.88                                                                                   | 1727A    | 0.82                                                                                   |    | 1573  | 1.32     | N.D.                                           | 1727A               | 1.57     | N.D.                                           |                     |
| 1574     | 1.07                                                                                   | 1728A    | 0.91                                                                                   |    | 1574  | 1.62     | N.D.                                           | 1728A               | 0.70     | N.D.                                           |                     |
| 1575     | 0.92                                                                                   | 1729     | 0.64                                                                                   |    | 1575  | 2.02     | N.D.                                           | 1729                | 1.05     | N.D.                                           |                     |
| 1577     | 0.67                                                                                   | 1730     | 0.69                                                                                   |    | 1577  | N.D.     | N.D.                                           | 1730                | 1.06     | N.D.                                           |                     |
| 1578     | 0.67                                                                                   | 1731     | 0.65                                                                                   |    | 1578  | 0.50     | N.D.                                           | 1731                | 0.88     | N.D.                                           |                     |
| 1604     | 0.76                                                                                   | 1732     | 0.73                                                                                   |    | 1604  | 0.36     | N.D.                                           | 1732                | 0.01     | N.D.                                           |                     |
| 1715     | <sup>1</sup> ND                                                                        | 1734     | 0.94                                                                                   |    | 1715  | 0.70     | N.D.                                           | 1734                | 1.98     | N.D.                                           |                     |
| 1716     | 0.62                                                                                   | 1812     | 0.80                                                                                   |    | 1716  | 0.38     | N.D.                                           | 1812                | N.D.     | N.D.                                           |                     |
| 1717     | 0.66                                                                                   | 1813     | 0.72                                                                                   |    | 1717  | 0.62     | N.D.                                           | 1813                | 0.49     | N.D.                                           |                     |
| 1733     | 0.49                                                                                   | 1857     | <sup>1</sup> ND                                                                        |    | 1733  | 1.62     | N.D.                                           | 1857                | N.D.     | N.D.                                           |                     |
| 1714A    | 0.50                                                                                   | 1858     | <sup>1</sup> ND                                                                        |    | 1714A | 2.70     | N.D.                                           | 1858                | N.D.     | N.D.                                           |                     |
| 1716A    | 0.60                                                                                   | 1814     | <sup>1</sup> ND                                                                        |    | 1716A | 0.45     | N.D.                                           | 1814                | 0.20     | N.D.                                           |                     |
| 1718A    | 0.60                                                                                   | 1x35     | 0.98                                                                                   |    | 1718A | 0.46     | N.D.                                           | 1x35                | 0.19     | N.D.                                           |                     |

<sup>1</sup> All specimens were solution-treated at 2150° F. for 1 hour, water quenched, and aged at 1400° F. 8 hours, except for the "21-4N" steel, which was aged for 16 hours.

N. D.—Not determined.

<sup>1</sup> Not determined.<sup>2</sup> Estimated.

TABLE IV.—RESULTS OF HARDNESS TESTS

| Heat No. | Compositional variable(s) | Hardness (Rockwell "C") | Solution treated <sup>1</sup> | Solution treated plus aged at 1,400° F. 8 hr. |
|----------|---------------------------|-------------------------|-------------------------------|-----------------------------------------------|
| 3230     | 0.20% C                   | 1                       | 8                             |                                               |
| 3229     | 0.29% C                   | 9                       | 12                            |                                               |
| 3103     | 0.36% C                   | 8                       | 20                            |                                               |
| 3168     | 0.45% C                   | 14                      | 18                            |                                               |
| 3169     | 0.71% C                   | 20                      | 22                            |                                               |
| 3170A    | 1.00% C                   | 16                      | 21                            |                                               |
| 3260     | No B                      | 15                      | 17                            |                                               |
| 3261     | No Cb, No B               | 12                      | 14                            |                                               |

<sup>1</sup> 2150° F. 1 hour, water-quench.

From the foregoing results, it is apparent that the preferred steels of our invention exhibit a weight loss, after immersion in molten lead oxide for 1 hour at 1675° F., of less than two-thirds that exhibited by the comparison steel "21-4N." Table II shows the effect of carbon on the lead oxide corrosion resistance, a maximum in such resistance being had at a carbon content of about 0.38% or 0.40%. Further inspection of data on Heat Nos. 1718A, 1716, 1719A, and 1720 in Table II shows the effect of the boron content on the lead oxide corrosion resistance. Table II further shows the effect on the lead oxide corrosion resistance that is obtained when columbium is used.

Table III shows that, unexpectedly, the creep strength reaches a maximum at about 0.38% or 0.40% carbon, which is the carbon range providing maximum resistance to lead-oxide corrosion. With such a carbon content it is possible to obtain a steel that closely approximates the known "21-4N" steel in creep strength, yet is considerably superior in its resistance to corrosion by lead oxide. This is especially remarkable because, as aforesaid, the "21-4N" steel has never, among the iron-base materials that have sufficient all-around oxidation resistance and high temperature creep strength to be useful in automotive and other internal-combustion-engine valves, been hitherto surpassed in lead oxide corrosion resistance. Moreover, comparison of Heat No. 1714A with Heat Nos. 1716 and 1718A reveals that creep strength can be obtained without any boron additions, but Heat Nos. 1719A and 1720A show that a still further improvement in strength is obtained when, as is preferred, boron is added.

Table III and FIGURE 4 also show that favorable creep strength results can be obtained by the addition of titanium, tantalum, molybdenum, or tungsten in place of columbium, but not with vanadium, zirconium, or aluminum. Table III also shows that the creep strength may be improved by additions of copper (Heat No. 1814) or nitrogen (Heat No. 1X35).

As respects machining, the machinability of a steel in accordance with the invention was evaluated in direct comparison with the "21-4N" valve steel in a lathe cut-off operation. The steel thus tested constitutes a preferred composition: 0.36% carbon, 6.03% manganese, 0.05% sulfur, 0.007% phosphorus, 0.07% silicon, 19.51% chromium, 5.84% nickel, 0.12% columbium, 0.002% boron, 0.07% nitrogen, balance iron. A standard AISI Type M1 high speed tool was used to cut off one-inch diameter bar stock of each steel in the solution-treated-and-aged condition. The tooling and machining conditions were as follows:

#### MACHINING CONDITIONS

|                |                                                                                                          |
|----------------|----------------------------------------------------------------------------------------------------------|
| Lathe          | American P a c e m a k e r<br>14 x 30" (equipped with a variable-speed drive for spindle-speed control). |
| Spindler speed | 150 r.p.m.                                                                                               |
| Cross feed     | 0.00315 in. per revolution.                                                                              |
| Coolant        | A proprietary hydrocarbon-type coolant of the kind well known to those skilled in the art.               |

#### TOOLING

|                    |                 |
|--------------------|-----------------|
| Tool material      | AISI type M1    |
| Tool blank size    | in. 6 x 1 x 1/8 |
| Tool geometry:     |                 |
| 5 Rake angle       | degrees 0       |
| Front relief angle | do 11.5         |
| Side relief angle  | do 3            |
| Nose angle         | do 11.5         |

10 The tool used to cut "21-4N" steel failed before even one cut was completed. In contrast, the tool used to cut the steels of this invention was still cutting satisfactorily after 32 cuts, when the test was discontinued.

15 Additional data demonstrating that the preferred steel of our invention is superior to "21-4N" steel in hot-workability is presented in the following Tables V and VI. Said preferred steel had the composition of Heat No. 1604 in Table II and the "21-4N" steel had the composition given in that table. One-inch-diameter bars of each steel were 20 heated to 2150° F. and then hot-rolled to flats 1/8-inch thick, using a substantially identical pass schedule. The roll-separating force and the exit thickness after each 25 pass were determined, and the thickness reduction achieved in each pass was calculated. Table V presents the data in the order in which they were obtained, and Table VI shows the relationship between roll-separating force and thickness reduction achieved for each of the steels.

TABLE V.—HOT-WORKABILITY TESTS

| Pass No. | Exit thickness, inch    |                         | Thickness reduction, percent | Roll-separating force, 1,000 lb. |
|----------|-------------------------|-------------------------|------------------------------|----------------------------------|
|          | Our steel "21-4N" steel | Our steel "21-4N" steel |                              |                                  |
|          | Our steel "21-4N" steel | Our steel "21-4N" steel |                              |                                  |
| 1        | 0.729                   | 0.728                   | 27                           | 16                               |
| 2        | 0.628                   | 0.630                   | 13                           | 10                               |
| 3        | 0.486                   | 0.485                   | 23                           | 18                               |
| 4        | 0.356                   | 0.388                   | 21                           | 22                               |
| 5        | 0.258                   | 0.262                   | 33                           | 44                               |
| 6        | 0.135                   | 0.140                   | 48                           | 98                               |
|          |                         |                         | 47                           | 140                              |

TABLE VI.—HOT-WORKABILITY-COMPARISON OF THICKNESS REDUCTION AND ROLL-SEPARATING FORCE

| Thickness reduction, percent | Our steel                  |                              | "21-4N" steel              |                              |
|------------------------------|----------------------------|------------------------------|----------------------------|------------------------------|
|                              | Roll-separating force, lb. | Thickness reduction, percent | Roll-separating force, lb. | Thickness reduction, percent |
| 13                           | 10,000                     | 13                           | 16,000                     |                              |
| 21                           | 22,000                     | 19                           | 24,000                     |                              |
| 23                           | 18,000                     | 24                           | 28,000                     |                              |
| 27                           | 16,000                     | 27                           | 20,000                     |                              |
| 33                           | 44,000                     | 33                           | 60,000                     |                              |
| 48                           | 98,000                     | 47                           | 140,000                    |                              |

50 From table VI it will be seen that in each case with the "21-4N" steel it required a greater roll-separating force to achieve a given amount of thickness reduction.

55 Further data demonstrating the improved workability of preferred steels in accordance with the instant invention is presented below.

60 The hot ductility of a preferred steel in accordance with our invention, in comparison with that of the known "21-4N" steel, was further evaluated in an elevated-temperature tension-impact test. In this test, cylindrical button-head specimens (0.375-inch-diameter by 0.8125-inch-long gage section) were heated to a test temperature, rapidly transferred to an impact machine with appropriate special fixtures, and then broken in tension under impact loading. The striking hammer weighed 60 pounds and was dropped from a height of 48 inches. The initial strain rate achieved in this test is about 256 in./in./sec., which is comparable to that which occurs during hammer-forging operations. The primary criterion for evaluating results in 65 this test is the fracture ductility, which is expressed as the percent reduction of area of the test specimen, higher percentages being more favorable. The force in foot-pounds required to break the specimen is also measured; in this test, lower numbers indicate superior ductility and work- 70 ability.

The two steels tested in this way had the following chemical compositions:

HEAT NO. 70413

|    |       |
|----|-------|
| C  | 0.36  |
| Mn | 6.03  |
| Si | 0.07  |
| S  | 0.050 |
| P  | 0.007 |
| Cr | 19.51 |
| Ni | 5.84  |
| Cb | 0.12  |
| B  | 0.002 |
| N  | 0.07  |

## "21-4N" STEEL

|    |                   |
|----|-------------------|
| C  | 0.53              |
| Mn | 9.28              |
| Si | 0.20              |
| S  | 0.070             |
| P  | 0.020             |
| Cr | 20.55             |
| Ni | 3.67              |
| Cb | <sup>1</sup> N.A. |
| B  | <sup>1</sup> N.A. |
| N  | 0.39              |

<sup>1</sup> None added.

Duplicate as-rolled specimens of each steel were tested at 2390° F., 2300° F., 2250° F., 2200° F., 2150° F., and 1800° F. Heating temperatures were the same as the test temperatures in each case, except for the tests at 1800° F., for which the specimens were first heated to 2150° F., and then cooled to 1800° F. being tested. The results of these tests are presented below in Table VII.

TABLE VII.—RESULTS OF TENSION-IMPACT TESTS

| Heating tem-<br>perature, ° F. | Test tempera-<br>ture, ° F. | Reduction of area,<br>percent |         | Rupture strength,<br>ft.-lb. |         |
|--------------------------------|-----------------------------|-------------------------------|---------|------------------------------|---------|
|                                |                             | 70413                         | "21-4N" | 70413                        | "21-4N" |
| 2,390                          | 2,390                       | 57                            | 34      | 93                           | 74      |
| 2,300                          | 2,300                       | 67                            | 63      | 119                          | 131     |
| 2,250                          | 2,250                       | 75                            | 67      | 141                          | 142     |
| 2,200                          | 2,200                       | 81                            | 76      | 151                          | 161     |
| 2,150                          | 2,150                       | 83                            | 80      | 156                          | 173     |
| 2,150                          | 1,800                       | 68                            | 55      | 172                          | 187     |

The above results indicate that the preferred steel of our invention is superior in hot workability, as respects both mill processing and valve manufacture. A hot-working temperature of about 2150° F. to 2250° F. appears most favorable.

There are other properties that may prove important in a valve steel. Among these are (1) tensile strength at room temperature and elevated temperature, (2) Charpy V-notch impact strength, (3) amenability to hardfacing, and (4) flash-weldability. Preferred steels of our invention exhibit at least satisfactory properties in the above respects. In room-temperature Charpy V-notch impact tests, the steel of Heat No. 70413 had impact values of 75

and 62 ft.-lb. in the solution-treated-and-aged condition, as compared with values of 4 and 5 ft.-lb. for the "21-4N" steel with which it was compared.

While we have shown and described certain embodiments of our invention, we intend to cover as well any change or modification therein which may be made without departing from the spirit and scope of the invention.

What is claimed is:

1. An austenitic stainless steel characterized by good high-temperature creep strength along with good hardness and formability consisting essentially of, in percent, about .22 to .5 carbon, 16 to 22 chromium, .05 to .25 silicon, 4 to 15 nickel, 2 to 8 manganese, with the combination of manganese plus nickel ranging from 8 to 20, up to .025 boron, up to .25 sulfur, up to .25 nitrogen, with the combination of carbon plus nitrogen ranging from .25 to .6, up to 3 copper, .02 to .75 of at least one element selected from the group consisting of columbium, molybdenum, tungsten, titanium and tantalum, and the balance iron, said stainless steel being fully austenitic and substantially free of ferrite.

2. The stainless steel of claim 1 further characterized by boron of .00005 to .025.

3. An austenitic stainless steel characterized by good high-temperature creep strength along with good hardness and formability consisting essentially of, in percent, about .22 to .5 carbon, 16 to 22 chromium, .05 to .25 silicon, 4 to 15 nickel, 2 to 8 manganese, with the combination of manganese plus nickel of 8 to 20, up to .025 boron, up to .25 sulfur, up to .25 nitrogen, with the combination of carbon plus nitrogen of .25 to .6, up to 3 copper, .05 to .25 columbium, and the balance iron, said stainless steel being fully austenitic and substantially free of ferrite.

4. The stainless steel of claim 3 further characterized by tantalum of .005 to .25.

## References Cited

## UNITED STATES PATENTS

|           |         |             |           |
|-----------|---------|-------------|-----------|
| 2,429,800 | 10/1947 | Briggs      | 75—128    |
| 2,495,731 | 1/1950  | Jennings    | 75—128    |
| 2,657,130 | 10/1953 | Jennings    | 75—128    |
| 2,671,726 | 3/1954  | Jennings    | 75—128    |
| 2,745,777 | 5/1956  | Clarke      | 75—128 XR |
| 2,799,577 | 7/1957  | Schempp     | 75—128    |
| 2,839,391 | 6/1958  | Loveless    | 75—128 XR |
| 2,892,703 | 6/1959  | Furman      | 75—128    |
| 3,152,934 | 10/1964 | Lula et al. | 75—128 XR |
| 3,310,396 | 3/1967  | Hochmann    | 75—128    |

## FOREIGN PATENTS

|         |        |                |
|---------|--------|----------------|
| 831,728 | 3/1960 | Great Britain. |
| 12,814  | 7/1963 | Japan.         |
| 12,502  | 8/1962 | Japan.         |

55 HYLAND BIZOT, Primary Examiner.

P. WEINSTEIN, Assistant Examiner.